

Sept. 20, 1927.

S. A. NEIDICH

1,643,080

PROCESS OF FORMING COLLOID PRODUCTS

Filed March 3, 1926

FIG. I.



FIG. II.



FIG. III.



FIG. IV.



FIG. V.



INVENTOR:

SAMUEL A. NEIDICH,  
by Arthur E. Paig,  
Secretary.

## UNITED STATES PATENT OFFICE.

SAMUEL A. NEIDICH, OF EDGEWATER PARK, NEW JERSEY.

## PROCESS OF FORMING COLLOID PRODUCTS.

Application filed March 3, 1926. Serial No. 91,962.

My invention is applicable in the manufacture of filaments by projecting viscose (cellulose sulphocarbonate) through orifices into baths containing chemicals which coagulate the viscose as a semi-solid impure cellulose hydrate of sufficient strength to be manipulated in the subsequent operations of dyeing, drying, and weaving or braiding the same. Ordinarily, filaments projected 5 through circular orifices and thus treated are solid cylinders of substantially uniform diameter and smooth exterior when dried. However, the purpose and effect of this invention is to produce a solid substantially 10 uniform cylindrical filament surrounded by a tubular sheath which is crinkled so that its exterior surface presents numerous facets for reflection of light so as to have a scintillating effect, which is particularly desirable 15 in the formations of braids, cords, etc., used in the millinery trade.

As hereinafter described; my invention includes the extrusion of primarily solid filaments of viscose, through suitable spinners, into a coagulating or precipitating medium, of such character as to immediately coagulate the exterior portion thereof, to such depth as to form what may be termed a skin, with the effect that, as the coagulation 20 and reversion of the viscose within such skin proceeds, such stresses are created that, ultimately, the core comprising the entire substantially cylindrical body of the filament, within such skin, at some stage in its 25 dehydration shrinks in diameter to such an extent as to pull loose from the skin, leaving the latter as a tubular sheath covering such cylindrical core throughout the length of the latter. However, during the desiccation 30 of the structure as a whole, said sheath shrivels so that its exterior surface becomes crinkled and affords numerous irregular facets for reflection of light as aforesaid.

My invention includes the various novel 45 features of procedure hereinafter more definitely specified.

I have found that the effect aforesaid is producible by certain relations of the factors of strength of the precipitating bath, the speed of traverse of the filament through 50 bath and time of exposure of the filament to the action of the bath.

Ordinarily, aqueous solutions containing eight percent of sulphuric acid or five percent 55 of hydrochloric acid are considered strong coagulating baths and are commonly

used for production of what are termed artificial silk filaments. However, it may be observed in the example of my invention hereinafter set forth that the acid strength of 60 the bath is more than double such ordinary baths.

With baths of that character, substantially all of the sulphur primarily chemically combined with the cellulose in viscose is released 65 as free sulphur and is occluded in the mass of cellulose hydrate, forms a dull yellow white surface upon the filament and renders the latter weak and brittle. It is practically impossible to more than partially remove 70 sulphur and its derivatives from such cellulose hydrate by any ordinary process. However, I have discovered that if any suitable coagulating bath is made to include  $PO_4$  ions; filaments of cellulose hydrate 75 formed by coagulating filaments in such baths are practically self-cleansing because the sulphur derivatives are thereby rendered soluble in the bath and automatically eliminated from the filaments. Such ions 80 may be added to or produced in such baths in any convenient form or manner. However, trisodium phosphate ( $Na_3PO_4$ ) is a cheap vehicle for such ions and may be used in aqueous solution. 85

Therefore, in one exemplification of my invention, I form a viscose precipitating bath of water containing sixteen and one half percent of  $H_2SO_4$ , in association with one half of one percent of  $PO_4$  ions, measured as  $PO_4$ , and cause the filaments of viscose containing twelve per cent. of cellulose to traverse such bath submerged in a path therethrough three and one half feet long and at the rate of one hundred twenty feet 90 per minute; so that the time of subjection of each portion of the filament to such bath is one and three quarter seconds. However, with a viscose containing fourteen percent, cellulose, with an alkalinity of 3.7 percent, 100 and tri-sodium phosphate content of .42 of the cellulose weight, filaments thereof of 300 denier are precipitated in the manner characteristic of this invention by submersion in a path but one-half inch long in a bath 105 containing 14.7 percent sulphuric acid and one-half percent, tri-sodium phosphate at a temperature of 70° C.

Although the peculiar effect aforesaid may be observed with a filament of three 110 hundred denier, it is markedly characteristic of filaments between six hundred and one

thousand denier and I prefer to utilize the same in filaments of nine hundred denier. It being noted that ordinary viscose contains but seven or eight percent of cellulose and is precipitated by an ordinary bath containing from eight to ten percent sulphuric acid; it is obvious that my invention is characterized both by the inclusion of an abnormally large percentage of cellulose in the viscose and by inclusion of an abnormally large percentage of acid in the precipitating bath. Although the required acid content of the bath varies inversely with the cellulose content of the viscose, as indicated by the two examples aforesaid, it is characteristic of my invention that the acidity of the precipitation bath shall be at least fifty percent greater than is ordinarily employed.

20 In said drawings: Fig. I is a perspective view of a piece of a finished product of my invention.

Fig. II is a fragmentary longitudinal sectional view of an extruded viscose filament before coagulation.

Fig. III is a sectional view similar to Fig. II but indicating the coagulation of the exterior of said filament to form the skin aforesaid.

30 Fig. IV is a sectional view, similar to Figs. II and III but showing the core of the filament shrunken to such an extent as to be separated from its skin.

Fig. V is a fragmentary sectional view of the structure indicated in Figs. II to IV inclusive but in the final dessicated state and showing the core filament in elevation and the skin sheath thereof in section.

Referring to Fig. I; the complete product 40 of my invention is an artificial thread, which may be woven, braided, knitted or otherwise embodied in any suitable texture and which includes the substantially smoothly cylindrical solid core filament 1 with the outer continuous imperforate tubular sheath 2 enclosing said core in substantially coaxial spaced relation therewith but having a shriveled crinkled exterior affording multitudinous facets 3 adapted to reflect light with a scintillating effect.

Figs. II to V inclusive indicate steps in the production of such an artificial textile thread as indicated in Fig. I; by the exemplification of my invention above described.

55 Fig. II shows the solid homogeneous filament 4 of viscose, which, as extruded through a circular orifice, is substantially cylindrical and of homogeneous structure throughout its mass. Fig. III indicates the practically instantaneous effect upon the filament of Fig. II incident to its submersion in the bath above contemplated; which effect is the coagulation of the exterior of the filament 4 to such depth as to form what may be termed 60 a skin 5. As the coagulation and reversion

of the viscose within such skin proceeds, such stresses are created that, ultimately, the core comprising the entire substantially cylindrical body of the filament 4, within such skin 5, at some stage in its dehydration 70 shrinks in diameter to such an extent as to pull loose from the skin, as indicated in Fig. IV, leaving said skin 5 as a tubular sheath 2 covering such cylindrical core throughout the length of the latter. During 75 the continued desiccation of the structure as a whole, said sheath shrivels so that its exterior surface becomes crinkled as indicated at 2 in Figs. and V, and affords innumerable facets 3 for reflection of light, so as to have 80 the desired scintillating effect. At such final stage of its production, both the interior core 1 and exterior sheath 2 have, of course, shrunken to much smaller diameter 85 than the viscose filament from which they are formed. In fact an extruded viscose filament may shrink to one half its original diameter.

It is most economical to produce such threads in the least possible time of use of the apparatus employed and, therefore, it is desirable to run the extruded filament 4 through the bath at high speed as in the example above set forth. However, the desired effect may be attained in a somewhat weaker bath by longer subjection of the filament thereto; provided that the coagulating action thereof is strong enough to produce the skin effect described.

Moreover, although I prefer to include 100  $\text{PO}_4$  ions in the bath to avoid the necessity for using other desulphurizing methods and means to cleanse the product; of course, threads of the double character above contemplated may be produced in baths which do not contain  $\text{PO}_4$  ions, and such threads be subsequently desulphurized by any of the ordinary methods and means, well known in the art.

Furthermore, although I prefer to form 110 such threads from the thiocarbonate of cellulose, known as viscose, as above described; containing about twelve per cent of cellulose, in hydrated form; there are at least four other methods of producing artificial colloid filaments in which my invention may be employed to wit, first, in the manufacture of filaments from nitro-cellulose by what is known as the Chardonnet methods and means; second, in what is known as the cuprammonium process, whereby filaments are formed from a solution of cellulose in an ammoniacal copper oxide; third, in the formation of filaments from a solution of cellulose zinc chloride; and fourth, in the formation of filaments from acetic anhydride. Each of said processes and the methods and means for effecting the same are well known to those skilled in the art and, therefore, my invention may be applied thereto, in 120 125 130

- each case, by using such increased strength of the coagulating or precipitating medium that the ordinary purpose and effect of gradually coagulating the extruded filament throughout its mass so as to leave the latter of uniform and unitary composition, which is characteristic of the ordinary processes, are defeated by the instantaneous production of a substantially hard and tough skin upon the extruded filament capable of resisting the shrinkage of the gelatinous mass which it incloses; so that the subsequent desiccation of the latter causes it to separate from such skin.
- 15 Therefore, I do not desire to limit myself to the precise details of procedure herein set forth, as it is obvious that various modifications may be made therein without departing from the essential features of my invention as defined in the appended claims.
- I claim:
1. The process of forming an artificial textile thread including a solid core filament and an outer tubular sheath, encasing said core, which consists in extruding a colloid including hydrated cellulose, through a circular orifice, into a coagulating medium comprising a bath of aqueous liquid containing sixteen and one-half per cent of sulphuric acid, associated with one-half per cent of  $\text{PO}_4$  ions; allowing each portion of said filament to remain submerged in said bath until the exterior thereof is coagulated to form a skin, primarily in unitary relation with the mass of colloid within it; continuing the reversion and elimination of moisture from said colloid until the core mass within said skin separates from the latter and forms a substantially smoothly cylindrical filament, and said skin forms an outer continuous imperforate tubular sheath, radially separated from said core, but in substantially coaxial, spaced, relation therewith, and having a shriveled crinkled exterior affording multitudinous facets adapted to reflect light with a scintillating effect.
  2. The process of forming an artificial textile thread including a solid core filament and an outer tubular sheath, encasing said core, which consists in extruding a colloid including hydrated cellulose, through a circular orifice, into a coagulating medium comprising a bath of aqueous liquid containing an acid, associated with  $\text{PO}_4$  ions; said bath being of at least fifty per cent greater acidity than is ordinarily employed to produce a solid filament; allowing each portion of said filament to remain submerged in said bath until the exterior thereof is coagulated to form a skin, primarily in unitary relation with the mass of colloid within it; continuing the reversion and elimination of moisture from said colloid until the core mass within said skin separates from the latter and forms a distinct filament, and said skin forms an outer continuous tubular sheath, radially separated from said core, but in substantially coaxial relation therewith, and having a shriveled crinkled exterior affording multitudinous facets adapted to reflect light with a scintillating effect.
  3. The process of forming an artificial textile thread including a solid core filament and an outer tubular sheath, encasing said core, which consists in extruding a colloid including more than eight per cent of hydrated cellulose, into a coagulating medium comprising a bath of aqueous liquid containing sulphuric acid, associated with  $\text{PO}_4$  ions; said bath being of at least fifty per cent greater acidity than is ordinarily employed to produce a solid filament; allowing each portion of said filament to remain submerged in said bath until the exterior thereof is coagulated to form a skin, primarily in unitary relation with the mass of colloid within it; continuing the reversion with the mass of moisture from said colloid until the core mass within said skin separates from the latter and forms a distinct filament, and said skin forms an outer continuous tubular sheath, radially separated from said core, but in substantially coaxial relation therewith, and having a shriveled crinkled exterior affording multitudinous facets adapted to reflect light with a scintillating effect.
  4. The process of forming an artificial textile thread including a solid core filament and an outer tubular sheath, encasing said core, which consists in extruding a colloid filament including more than eight per cent of hydrated cellulose, into a coagulating medium comprising a bath of aqueous liquid containing sulphuric acid; said bath being of at least fifty per cent greater acidity than is ordinarily employed to produce a solid filament; allowing each portion of said filament to remain submerged in said bath until the exterior thereof is coagulated to form a skin, primarily in unitary relation with the mass of colloid within it; continuing the reversion and elimination of moisture from said colloid until the core mass within said skin separates from the latter and forms a distinct filament, and said skin forms an outer continuous tubular sheath, radially separated from said core, but in substantially coaxial relation therewith, and having a shriveled crinkled exterior affording multitudinous facets adapted to reflect light with a scintillating effect.
  5. The process of forming an artificial textile thread including a solid core filament and an outer tubular sheath, encasing said core, which consists in extruding a colloid filament into a coagulating medium; said bath being of at least fifty per cent greater acidity than is ordinarily employed to produce a solid filament; allowing each por-

tion of said filament to remain in said medium until the exterior thereof is coagulated to form a skin, primarily in unitary relation with the mass of colloid within it; continuing the elimination of moisture from said colloid until the core mass within said skin separates from the latter and forms a distinct filament, and said skin forms an outer continuous tubular sheath, separated from, but encasing, said core, and having a crinkled exterior adapted to reflect light with a scintillating effect.

6. The process of forming an artificial textile thread including a solid core filament and an outer tubular sheath, encasing said core, which consists in extruding a colloid

as an initially unitary filament; coagulating the exterior thereof to form a skin, primarily in unitary relation with the mass of colloid within it, by submerging it in a bath of at least fifty per cent greater acidity than an ordinary viscose precipitating bath; and continuing the coagulation of said colloid until the core mass within said skin separates from the latter and forms a distinct filament, and said skin forms an outer continuous tubular sheath.

In testimony whereof, I have hereunto signed my name at Burlington, New Jersey, this twenty-seventh day of January, 1926.

SAMUEL A. NEIDICH.

tion of said filament to remain in said medium until the exterior thereof is coagulated to form a skin, primarily in unitary relation with the mass of colloid within it; continuing the elimination of moisture from said colloid until the core mass within said skin separates from the latter and forms a distinct filament, and said skin forms an outer continuous tubular sheath, separated from, but encasing, said core, and having a crinkled exterior adapted to reflect light with a scintillating effect.

6. The process of forming an artificial textile thread including a solid core filament and an outer tubular sheath, encasing said core, which consists in extruding a colloid

as an initially unitary filament; coagulating the exterior thereof to form a skin, primarily in unitary relation with the mass of colloid within it, by submerging it in a bath of at least fifty per cent greater acidity than an ordinary viscose precipitating bath; and continuing the coagulation of said colloid until the core mass within said skin separates from the latter and forms a distinct filament, and said skin forms an outer continuous tubular sheath.

In testimony whereof, I have hereunto signed my name at Burlington, New Jersey, this twenty-seventh day of January, 1926.

SAMUEL A. NEIDICH.

**CERTIFICATE OF CORRECTION.**

Patent No. 1,643,080.

Granted September 20, 1927, to

SAMUEL A. NEIDICH.

It is hereby certified that error appears in the printed specification of the above numbered patent requiring correction as follows: Page 2, line 79, after "Figs." insert the numeral "1"; page 3, lines 88 and 89, claim 3, strike out the words "with the mass" and insert instead the words "and elimination"; and that the said Letters Patent should be read with these corrections therein that the same may conform to the record of the case in the Patent Office.

Signed and sealed this 11th day of October, A. D. 1927.

Seal.

M. J. Moore,  
Acting Commissioner of Patents.

**CERTIFICATE OF CORRECTION.**

Patent No. 1,643,080.

Granted September 20, 1927, to

**SAMUEL A. NEIDICH.**

It is hereby certified that error appears in the printed specification of the above numbered patent requiring correction as follows: Page 2, line 79, after "Figs." insert the numeral "1"; page 3, lines 88 and 89, claim 3, strike out the words "with the mass" and insert instead the words "and elimination"; and that the said Letters Patent should be read with these corrections therein that the same may conform to the record of the case in the Patent Office.

Signed and sealed this 11th day of October, A. D. 1927.

Seal.

**M. J. Moore,  
Acting Commissioner of Patents.**